

# UNITED STATES PATENT OFFICE.

ARNOLD ERLENBACH, OF DESSAU, GERMANY, ASSIGNOR TO ACTIEN GESELLSCHAFT  
FÜR ANILIN FABRIKATION, OF BERLIN, GERMANY.

## PROCESS OF DYEING HAIRS, FURS, AND THE LIKE.

992,947.

No Drawing.

Specification of Letters Patent. Patented May 23, 1911.

Application filed April 9, 1910. Serial No. 554,515.

To all whom it may concern:

Be it known that I, ARNOLD ERLENBACH, a subject of the King of Bavaria, residing at Dessau, Germany, my post-office address 5 being Schillerstrasse 5, Dessau, Germany, have invented certain new and useful Improvements in Processes of Dyeing Hairs, Furs, and the Like, of which the following is a specification.

10 My present invention relates to an improved process of dyeing hairs, furs and the like.

In dyeing hairs, furs and the like black shades aromatic diamins and more especially 15 para-phenylenediamin have been used in combination with an oxidizing agent, such as hydrogen peroxid. The latter para-diamin has extensively been applied in dyeing furs and the furs dyed with this base 20 whether with or without the aid of a metal salt as a mordant exhibit a coal black shade, but the shade lacks the bluish tint generally demanded and imparting a bloom to the dyeing. In order to improve the tints 25 obtained by the foregoing way one has also used a mixture of para-phenylenediamin and of certain meta-diamins, such as for instance meta-phenylenediamin or meta-to- 30 luylendiamin. Although by oxidation of these bases together with para-phenylenediamin somewhat more bright and more blue-black tones are obtainable, the dyeings are 35 unstable; when the dyed goods are stored the dyeing assumes after some time a red- brown shade. Now I have made the very 40 surprising observation that the aforesaid objections do not occur if instead of the above-named meta-diamins meta-diamino- anisol

(OCH<sub>3</sub> : NH<sub>2</sub> : NH<sub>2</sub> = 1:2:4)

or diaminophenetol

(OC<sub>2</sub>H<sub>5</sub> : NH<sub>2</sub> : NH<sub>2</sub> = 1:2:4)

45 are used. Thus I obtain in this new manner on hairs, furs and the like bright blue-black tones of great stability. For instance I apply to the furs a solution which contains in suitable proportions para-phenylenediamin, 50 meta-diamino-anisol and a suitable oxidizing agent, such as hydrogen peroxid. Similar results are also obtained if according to 55 my new process a suitable derivative of para-phenylenediamin, such as para-toluylenediamin, chloro-para-phenylenediamin, methoxy-para-phenylenediamin and the like

are employed instead of para-phenylenediamin; thus I produce very useful, brilliant blue-black dyeings of a great stability.

The following examples illustrate my invention, the parts being by weight:

1. 3 parts of para-phenylenediamin and 2 parts of diamino-anisol are dissolved in 500 parts of boiling hot water and 400 parts of cold water and 100 parts of hydrogen peroxid of 3 per cent. strength are added. The previously washed furs are introduced into the bath, cooled to 30-35° C. and handled therein for 6-12 hours; they are then washed and dried. In this manner intense blue 65 black colored furs are obtained.

2. The washed furs are mordanted with a solution of pyrolignite of iron (containing 20 grams of the commercial "pyrolignite of iron" per liter) over night; they are 75 then washed and dyed for about 12 hours in a bath which contains per liter 4.2 parts of para-phenylenediamin, 2.8 parts of diamino-anisol and 140 parts of hydrogen peroxid of 3 per cent. strength. The dyeings obtained according to this example are 80 more deep black than those obtained according to Example 1, but possess likewise the beautiful bluish shade.

Of course my present invention is not limited to the foregoing examples or to the details given therein. Thus for instance instead of diamino-anisol the corresponding diamino-phenetol may be employed; furthermore for para-phenylenediamin 90 may be substituted chloro-para-phenylenediamin, para-toluylenediamin, methoxy-para-phenylenediamin and the like. It is obvious that in using such another para-diamin, or in substituting meta-diamino-phenetol for the meta-diamino-anisol employed in the above example, the proportions of the ingredients as well as the duration of the dyeing, or of the mordanting 95 process, may be varied in order to obtain the best results. Also the special conditions of the dyeing process, or of the mordanting process, depend to a great deal upon the special nature of the hairs or the furs, etc., 100 to be dyed as well as of the desired shade. Finally instead of hydrogen peroxid any 105 other oxidizing agent suitable for the purpose of my present invention may be used.

Having now described my invention and the manner in which it may be performed, 110 what I claim is,—

1. The hereinbefore-described process for

dyeing hirsutical material, which consists in applying to the hairs or furs or the like a solution containing an aromatic para-diamin of the general formula:

5



in which formula R means a substituent, an aromatic meta-diamin of the general formula:

2. The herein described process for dyeing hirsutical material, which consists in applying to the hirsutical material a solution containing para-phenylenediamin, meta-diamin-anisol and an oxidizing agent.

20

In testimony whereof I have hereunto set my hand in presence of two subscribing witnesses.

ARNOLD ERLENBACH.

Witnesses:

RUDOLPH FRICKE,  
ALBERT R. MORAWETZ.



in which formula R means an oxyalkyl group and an oxidizing agent.

10

15